# EUROPEAN PATENT SPECIFICATION

(11) **EP 2 229 468 B1**
(45) Date of publication and mention of the grant of the patent: **25.01.2017**
(21) Application number: 08860540.7
(22) Date of filing: 23.10.2008
(51) Int. Cl.: C23D 3/00, B05D 7/14

(54) **PROCESS FOR THE PRODUCTION OF ENAMELLED STEEL SHEET OR PART**
VERFAHREN ZUR HERSTELLUNG EINES EMAILLIERTEN STAHLBLECHES ODER TEILS
PROCESSUS POUR LA PRODUCTION D'UNE PLAQUE OU PIÈCE D'ACIER ÉMAILLÉE

(30) Priority: 13.12.2007 EP 07291521
(43) Date of publication of application: 22.09.2010
(73) Proprietor: ArcelorMittal, 1160 Luxembourg (LU)
(72) Inventor: LEVEAUX, Marc, F-59700 Marcq en Baroeul (FR); DUPREZ, Lode, B-9160 Lokeren (BE); GONZÁLEZ JIMÉNEZ, Javier, 9000 Gent (BE); GOUSSELOT, Philippe, F-57070 Metz (FR)
(74) Representative: Lavoix
(86) International application number: PCT/IB2008/002864
(87) International publication number: WO 2009/074854

(56) References cited:
- GB-A- 1 221 836
- US-A1- 2003 031 797

## Description

The present invention relates to a steel sheet or part whose composition is suitable for enamelling, and which is coated on one or both sides with a coating consisting of a matrix of polymer in which particles of non-oxide ceramic are homogeneously dispersed, and the use of this coated steel sheet or part for producing an enamelled steel sheet or part.

It also relates to a process for manufacturing a steel sheet or part coated with a layer of ground coat enamel and an optional further layer of white or light-coloured cover coat enamel having a high adhesion with respect to the steel.

The protection of metallic surfaces by application of a layer of enamel is well-known, and is widely used due to its resistance to high temperature and because it gives the surface a protection against chemical aggression.

Enameled products are thus widely used in different applications such as in washing machines, sanitary ware, cooking range, domestic appliances, as well as outside construction materials.

The conventional process for producing enamelled steel sheet with a high adhesion between the steel sheet and the enamel coating, comprises the application to the steel sheet of a layer of enamel containing adherence promoting oxides such as cobalt, nickel, copper, iron, manganese, antimony or molybdenum oxides. This kind of enamel is called "ground coat enamel".

The adhesion of the ground coat enamel on steel is obtained, by firing from 780 to 860°C during 3 to 8 min, via oxido-reduction chemical reaction between the elements of the steel, such as carbon, and adherence promoting oxides of the ground coat enamel.

However, the time and temperature required to fire the enamel do not match anymore with nowadays industrial requirements.

US2003/031797 already discloses a process for enamelling a metal part comprising applying a polymer emulsion and a liquid enamelling composition to avoid any degreasing operation. It is also known from GB1221836 to add non-oxide ceramic particles in polyarylene oxide polymers to control their tendency to sag under the conditions of coating and curing.

The purpose of the present invention is therefore to remedy the aforementioned drawbacks and to provide a process for producing an enamelled steel sheet or part, which allows a decrease of the consumption of energy by decreasing the firing temperature by 10 to 40°C compared with conventional firing temperatures, and an increase of the productivity by decreasing the firing time by 1 to 3 min compared with conventional firing times, while maintaining both a good adhesion and surface aspect of the enamel layer.

The object of the invention is therefore a process for enamelling a steel sheet or part comprising the steps consisting in:
- applying to one or both sides of a steel sheet whose composition is suitable for enamelling, a formulation layer comprising 0.008 to 5% by weight of particles of non-oxide ceramic whose melting point is above 600°C, an optional solvent, the balance being a polymer which, when heated from ambient temperature to 800°C in air, gets burned at more than 80% by weight at 440°C and is completely burned at 600°C,
- curing said layer so as to obtain a polymer coating in which the particles of non-oxide ceramic are homogeneously dispersed,
- optionally subjecting said coated steel sheet to a forming operation in order to obtain a part,
- applying to said polymer coating a layer of ground coat enamel, and optionally a further layer of white or light-coloured cover coat enamel, then
- subjecting said ground coat enamel and said optionally white or light-coloured cover coat enamel to a firing to obtain an enamelled steel sheet or part.

The process according to the invention is advantageous not only because a decrease of the firing temperature and time is achieved, but also because unfriendly environmental preparation of the steel sheet, before and after the application of the formulation, and before the enamelling, such as intensive pickling with acidic solutions and/or nickling, is not required.

A steel sheet or part whose composition is suitable for enamelling is defined according to the European standard EN 10209, and is characterized by a low-carbon content, generally less than 0.08% by weight, in order to avoid the formation of bubbles during the firing of the enamel. Thus, low carbon steel grade with a carbon content less than 0.08% by weight, ultra-low carbon steel grade with a carbon content less than 0.005% by weight and Ti-interstitial free steel with a carbon content less than 0.02% by weight may be considered to carry out the present invention.

A second object of the invention is a steel sheet or part coated on one or both sides with a coating consisting of a matrix of polymer in which particles of non-oxide ceramic are homogeneously dispersed, the coating weight of said particles being between 0.001 and 0.250 g/m², the melting point of said non-oxide ceramic being above 600°C, the composition of said steel sheet or part being suitable for enamelling, and said polymer, when heated from ambient temperature to 800°C in air, getting burned at more than 80% by weight at 440°C and being completely burned at 600°C.

Finally a third object of the invention is the use of said coated steel sheet or part for producing an enamelled steel sheet or part

After hot rolling and cold rolling, a steel sheet whose composition is suitable for enamelling, is simply degreased in order to remove all traces of lubricant, and is coated on one or both sides with a formulation layer comprising 0.008 to 5% by weight of particles of non-oxide ceramic whose melting point is above 600°C, an optional solvent, the balance being a polymer which, when heated from ambient temperature to 800°C in air, gets burned at more than 80% by weight at 440°C and is completely burned at 600°C.

The application of said formulation may be performed in a conventional manner, for example by dipping, roll coating, or spraying.

Then, said steel sheet coated with said formulation layer is cured so as to obtain a steel sheet coated with a polymer coating in which the particles of non-oxide ceramic are homogeneously dispersed.

Said polymer may be for example polyester, poly-acrylic, polyurethane, polyethylene, polypropylene, or the mixtures thereof.

In one embodiment of the invention, the polymer may be a radiation curable polymer, and the formulation is free of solvent.

The curing of said radiation curable polymer is thus performed by exposing the formulation layer to ionizing or actinic radiation.

The ionizing radiation may be electron beam, and the actinic radiation may be ultra-violet light.

In another embodiment of the invention, the polymer may be a thermal curable polymer. In this case, the formulation comprises a solvent. According to the invention, the solvent plays no active role during the formation of the polymer coating, and no structural element from the solvent is incorporated into the polymer.

The content of solvent and polymer in the formulation is selected to obtain a fluid formulation which may be easily applied to the steel sheet.

In addition, the solvent makes it easier to control the thickness of the coating. Indeed, a solvent-free formulation comprising a thermal curable polymer would be solid at ambient temperature, and should be applied to the steel sheet as liquid melted either by pre-heating and spraying it to the surface of said steel sheet, or by rubbing it against the pre-heated steel sheet. In these conditions, it would be difficult to have a homogeneous particle distribution and maintain a constant and thin thickness.

Thus, said formulation preferably comprises 0.008 to 5% by weight of said particles of non-oxide ceramic, 10 to 70% by weight of said thermally curable polymer, the balance of the composition being a solvent.

When the steel sheet is coated with said formulation layer, it is subjected to a heat treatment so as to cure the polymer, and completely evaporate the solvent.

The solvent has to be completely removed from the polymer coating, otherwise it will be difficult to avoid the dirtying of the coating surface, and the adhesion of the enamel with the steel sheet will be reduced or even prevented.

The heat treatment is performed by heating said steel sheet from ambient temperature to a temperature T1, and maintaining it at this temperature T1 for a time t1. It may be achieved by induction curing or by blowing hot air.

Preferably, the temperature T1 is between 50 and 220°C, and the time t1 between 5 s and 60 s. Above 220°C, the polymer may start to burn down before the application of the ground coat enamel, and there is a risk that the particles of non-oxide ceramic are not embedded anymore in the polymer, and are not homogeneously distributed on the surface of the steel sheet, leading to a smaller reduction of the firing time and temperature.

If the time t1 is above 60 s or if the temperature T1 is below 50°C, the process does not match with industrial requirements of productivity. However, if the time t1 is below 5 s, the drying and the curing of the layer will be insufficient.

The solvent may be an organic solvent, a hydro-organic solvent, or preferably water due to environmental purpose.

In both embodiments, a reduction of the firing time and temperature of the further enamel layer and an improved adhesion of the enamel to the entire surface of the steel sheet can only be reached if:
1) the amount of particles of non-oxide applied to the steel sheet is sufficient to react with the adherence promoting oxides of the ground coat enamel as will be seen later. Indeed, it is essential that the coating weight of said particles of non-oxide ceramic is more than 0.001 g/m². However, the coating weight is limited to 0.250 g/m², because the adhesion of the enamel is not improved anymore above 0.250 g/m², and the cost increases. More preferably, the coating weight of said particles of non-oxide ceramic is between 0.01 to 0.10 g/m².
2) the particles of non-oxide ceramic are homogeneously distributed on the surface of the steel sheet. The role of the polymer is to keep the particles of non-oxide ceramic homogeneously distributed on the steel surface, before the application of the enamel.

Preferably, the coating weight of the polymer coating, after heat treatment or exposure to ionizing or actinic radiation, is sufficient to provide the steel sheet with an effective temporary corrosion protection before the application of the ground coat enamel, but is low enough so that the polymer easily burns down during the firing of the enamel.

Thus, the coating weight of said polymer coating is preferably between 0.5 and 10.0 g/m², which corresponds to an amount of particles of non-oxide ceramic between 0.08 and 10% by weight. More preferably, the coating weight of the polymer is between 2.0 and 6.0 g/m².

Said formulation may also contain additives well known in the art to further enhance its properties: for example, surfactants to promote wetting of the surface of the steel sheet to be treated, antifoams, corrosion inhibitors, pigments or bactericides. All of these additives are generally used in relatively small amounts, usually less than 3% by weight with respect to the formulation.

After heat treatment or exposure to radiation, and before enamelling, the steel sheet can be subjected to a forming operation by stamping, drawing or bending, so as to obtain a part.

Preferably, the polymer coating is sufficiently lubricating to avoid the application of a further lubricant before the optional forming step. In this case, there is no need to degrease the polymer coated part before the application of the enamel.

However, if the polymer coating, itself, is not sufficiently lubricating, a lubricant can be added to the formulation in the range of 0.3 to 5% by weight with respect to the polymer. Below 0.3% by weight, the lubricating effect will not be sufficient to form the steel sheet without a prior lubricating operation by oiling for example, but above 5% by weight, there is a risk that the coating has a greasy appearance.

The lubricant may be for example a hydrocarbon wax, a vegetable wax such as carnauba wax, a mineral or synthetic oil, a vegetable or animal oil containing fatty acid esters, or fatty acid.

After heat treatment or exposure to radiation and the optional forming step, a layer of ground coat enamel is applied to the polymer coating, and is subjected to firing.

A ground coat enamel is a glass whose components are in the form of powder. Generally, it comprises 40 to 50% by weight of silica, 10 to 20% of boric oxide, 2 to 10% by weight of aluminium oxide, 0.5 to 4% by weight of transition metal oxides such as cobalt, nickel, iron, manganese, antimony and molybdenum oxides, the balance of the composition being alkaline oxides and alkaline-earth oxides. The transition metal oxides are called adherence promoting oxides, because they can be reduced by the elements of the steel such as carbon, and thus make the link between the steel sheet and the enamel.

The layer of ground coat enamel can be applied directly in powder form by dry electrostatic powdering, or in wet form after mixing with water, by spraying or dipping.

In the latter case, water is preferably completely evaporated before the firing step, by heating the layer of enamel from ambient temperature to a temperature T2, and maintaining it at this temperature T2 for a time t2.

The time t2 is preferably below 60 s to match with industrial requirements of productivity. That is the reason why the lower limit for the temperature T2 is preferably above 80°C. The time t2 is preferably above 5 s to insure a complete evaporation of water during the drying of the enamel. Otherwise, if the enamel layer is not completely dried before the firing, water will evaporate during the firing step, and the bonding of the enamel with the steel sheet will be impaired.

The temperature T2 is preferably limited to 120°C, to avoid bubble formation in the enamel layer during the evaporation of water, which would further impair the bonding of the enamel within the steel sheet.

The drying of the enamel in wet form may be performed by blowing hot air.

After the drying of the enamel in wet form, and before the firing of said dried enamel, the enamel may be cooled to ambient temperature. However, it is preferable to subject it to firing when it is still at said temperature T2 to save energy.

In both cases, before being fired, the layer of enamel is porous and contains generally 30 to 60% by volume of air.

The firing of the ground coat enamel comprises several steps, during which the steel sheet is subjected to heating either from ambient temperature or from the temperature T2.

Above 240°C, the polymer starts to burn down. That means that it is progressively degraded by the combination of heat and oxygen coming from air contained in the enamel layer, into carbon dioxide and water vapour which are released in the ambient atmosphere.

The inventors noticed that it is essential that more than 80% by weight of the polymer gets burned at 440°C, because if more than 20% by weight of polymer is not degraded before the enamel becomes a viscous liquid, there is a risk of adhesion problems of the enamel on the steel sheet, and of crater formation due to a huge release of gas bubbles during the firing of the enamel, leading to a bad surface aspect of the enamel coating.

At a temperature T3 which is conventionally between 450 and 600°C, the ground coat enamel starts to soften. and becomes a viscous liquid. The enamel layer is thus progressively changed from a porous layer into a continuous film, leading to a reduction of gaseous exchange. That is the reason why, the polymer has to be completely burned at 600°C, so as to avoid crater formation in the enamel coating due to release of gas bubbles, and adhesion problems of the enamel.

Then, as the temperature continues to increase, the particles of non-oxide ceramic and carbon coming from the steel reduce the transition metal oxides which are the most thermodynamically unstable oxides of the enamel, and give the adhesion of the enamel to the steel surface. The action of carbon is thus reinforced by the particles of non-oxide ceramic, which have the ability to compensate for the missing carbon of some kinds of steel, either nearly absent if ultra-low carbon steel is considered, or strongly bonded to titanium if titanium interstitial free steel is considered. As will be shown in the further examples, it has been observed that the firing temperature and time could be significantly reduced compared to the prior art.

Finally, the enamelled steel sheet is solidified by cooling to ambient temperature.

A non-oxide ceramic is a refractory material composed of a metal which is combined with carbon, nitrogen, boron, silicon or sulphur.

According to the invention, the melting point of the non-oxide ceramic has to be above 600°C, and preferably above 700°C, because it is essential to preserve the reduction ability of the particles of non-oxide ceramic during the firing step of the ground coat enamel. Indeed, at said temperature T3, a non-oxide ceramic having a melting point below 600°C would start to melt and be oxidised by air contained in the enamel layer, and would thus lose its ability to reduce the transition metal oxides.

The particles of non-oxide ceramic can thus be selected from the group consisting of nitrides, borides, silicides, sulphides, carbides, and the mixtures thereof, having a melting point above 600°C.

It can be for example, silicon nitride (Si₃N₄), boron nitride (BN), aluminium nitride (AlN), silicon carbide (SiC), boron carbide (B₄C), magnesium boride (MgB₂), titanium boride (TiB₂), zirconium boride (ZrB₂), molybdenum silicide (MoSi₂) or tungsten sulphide (WS₂).

The average diameter D50 of said particles of non-oxide ceramic is preferably between 0.01 and 3 µm, because when the average diameter D50 is more than 3 µm, the reactivity of the non-oxide ceramic towards transition metal oxides is not so high, and the reduction of firing time and temperature will be insufficient. On the other hand, below 0.01 µm, they are difficult to implement.

If a white or light-coloured surface aspect is required, a further layer of white or light-coloured cover coat enamel may be applied to the surface of the ground coat enamel. The firing of the layers of ground coat enamel and of white or light-coloured cover coat enamel can be performed either subsequently or simultaneously under the same conditions of firing temperature and time mentioned above.

The composition of white or light-coloured cover coat enamel is similar to that of ground coat enamel except that it comprises no transition metal oxides.

In the C.I.E. L.a.b. system adopted by CIE in 1976, a colour is represented by three numbers, which specify its position in a three-dimensional volume. The first number, the lightness L value, runs from 0 (black) to 100 (white), and defines how light or dark the colour is. The other numbers, a and b, give information about the colour from green to red, and from blue to yellow.

According to the invention, the lightness L of white or light coloured cover coat enamel is above 60.

After the firing, the thickness of the layer of ground coat enamel may be for example, between 80 and 150 µm if no further layer of white or light-coloured cover coat enamel is applied, and between 20 and 60 µm if a further layer of white or light-coloured cover coat enamel is applied, the thickness of said further layer being able to be between 80 and 120 µm.

The firing of the ground coat enamel, and of the further optional white or light-coloured cover coat enamel, may be performed in a conventional tunnel furnace having means for extracting fumes.

The invention will now be illustrated by examples given by way of nonlimiting indication.

Trials were carried out using samples coming from a steel sheet suitable for enamelling, referenced as DC03ED according to the standard EN10209 (also known as Solfer®).

The aim is to compare the adhesion of samples which were enamelled according to the invention with samples which were conventionally enamelled.

### 1- Production of conventionally enamelled steel sheets

After elimination of the protective oil from the surface of samples by conventional alkaline degreasing, a layer of conventional ground coat enamel referenced PP 12189, manufactured by Pemco International is applied to one side of a sample, in order to get an enamelled layer whose thickness is 110 µm after firing, that is about 400 g/m².

The enamelled samples are fired in a conventional furnace for enamelling at different firing temperatures and times, and the level of adhesion of the enamel layer is estimated according to the standard EN 10209, which defines a scale of five quotations, from 1 for an excellent adhesion to 5 for a bad adhesion. The results are shown in table I.

**Table I**

| Firing time (min) | Firing temperature (°C) | | | | | |
|---|---|---|---|---|---|---|
| | 800 | 810 | 820 | 830 | 840 | 860 |
| 2 | 5 | 4 | 4 | 3 | 2 | 1 |
| 2,5 | 4 | 3 | 3 | 2 | 1 | - |
| 3 | 4 | 3 | 3 | 2 | 1 | - |
| 3,5 | 3 | 2 | 2 | 1 | - | - |
| 4 | 3 | 2 | 1 | 1 | - | - |
| 4,5 | 2 | 2 | 1 | - | - | - |
| 5 | 1 | 1 | - | - | - | - |

| | | | | | | |
|---|---|---|---|---|---|---|
| (-): not tested | | | | | | |

### 2- Production of steel sheets enamelled according to the invention

Before enamelling, the samples are conventionally degreased by conventional alkaline solution in order to eliminate the protective oil from the surface.

Then, a layer of a formulation according to the invention is applied to one side of the samples.

Said formulation is prepared by mixing demineralised water, an aqueous acrylic polymer dispersion, referenced Prox AM355 from Protex-Synthron, and different kind of particles of non-oxide ceramic from H. C. Starck GmbH, as shown in table II. The content of water (including water coming from Prox AM355), acrylic polymer and non-oxide ceramic is expressed in % by weight with respect to the formulation.

**Table II**

| | Non-oxide ceramic | | | | | | | |
|---|---|---|---|---|---|---|---|---|
| | Si₃N₄ | TiB₂ | SiC | B₄C | BN | AlN | MoSi₂ | WS₂ |
| % of acrylic polymer | 14.24 | 14.24 | 14.27 | 14.25 | 14.27 | 14.26 | 14.19 | 14.11 |
| % of ceramic | 0.33 | 0.33 | 0.11 | 0.26 | 0.11 | 0.18 | 0.64 | 1.2 |
| % of water | 85.43 | 85.43 | 85.62 | 85.49 | 85.62 | 85.56 | 85.17 | 84.69 |
| Total | 100 | 100 | 100 | 100 | 100 | 100 | 100 | 100 |

The formulation coating weight applied to the samples is 4 g/m², wet.

The formulation layer is cured and completely dried by heating it from ambient temperature to 90°C, and maintaining it at 90°C for 30 s. When water is completely removed from the layer, the coating weight of the polymer coating is thus 0.6 g/m².

Then a layer of the same conventional ground coat enamel referenced PP 12189 previously used for producing conventional enamelled steel sheet, is applied to the polymer coating comprising the particles of non-oxide of ceramic. The application is performed in order to get an enamelled layer whose thickness is 110 µm after firing, that is about 400g/m².

The enamelled samples according to the invention are fired in a conventional furnace for enamelling at different firing times and temperatures, and the level of adhesion of the enamel layer is estimated according to the standard EN 10209. The results are shown in table III.

The surface aspect of each sample enamelled according to the invention is visually checked by an operator, and compared with the surface aspect of the samples conventionally enamelled. No change is observed, the surface aspect is good for each sample enamelled according to the invention.

**Table III**

| Kind of ceramic used | Time of firing (min) | Temperature of firing (°C) | | | |
|---|---|---|---|---|---|
| | | 800 | 810 | 820 | 830 |
| Si₃N₄ | 2 | - | - | 3 | - |
| | 2.5 | - | - | 2 | - |
| | 3 | - | 2 | 2 | - |
| | 3.5 | - | 2 | - | - |
| TiB₂ | 2 | - | - | 1 | - |
| | 2.5 | - | - | 1 | - |
| SiC | 2.5 | - | - | - | 1 |
| | 3 | - | 1 | - | - |
| B₄C | 2 | - | - | - | 1 |
| | 3 | - | - | 2 | - |
| | 3.5 | 2 | - | - | - |
| BN | 3 | - | - | 1 | - |
| | 3.5 | 1 | - | - | - |
| AIN | 2.5 | - | - | 2 | 1 |
| MoSi₂ | 3 | - | - | 1 | - |
| | 3.5 | 1 | - | - | - |
| WS₂ | 2.5 | - | - | 2 | - |
| | 3 | - | 2 | - | - |
| | 4 | 1 | - | - | - |

| | | | | | |
|---|---|---|---|---|---|
| (-): not tested | | | | | |

From the comparison of tables I and III, it can be observed that the use of a non-oxide ceramic according to the invention allows a decrease of the firing temperature and time.

## Claims

1. A steel sheet or part coated on one or both sides with a coating consisting of a matrix of polymer in which particles of non-oxide ceramic are homogeneously dispersed, the coating weight of said particles being between 0.001 and 0.250 g/m², the melting point of said non-oxide ceramic being above 600°C, the average diameter D50 of said particles being between 0.01 and 3 µm, the composition of said steel sheet or part being suitable for enamelling, and said polymer, when heated from ambient temperature to 800°C in air, getting burned at more than 80% by weight at 440°C and being completely burned at 600°C.

2. The steel sheet or part according to claim 1, wherein the coating weight of said particles of non-oxide ceramic is between 0.01 and 0.10 g/m².

3. The steel sheet or part according to claim 1 or 2, wherein the melting point of said non-oxide ceramic is above 700°C.

4. The steel sheet or part according to any one of claims 1 to 3, wherein said particles of non-oxide ceramic are selected from the group consisting of nitrides, borides, silicides, sulphides, carbides and the mixtures thereof.

5. The steel sheet or part according to any one of claims 1 to 4, wherein the coating weight of said polymer coating is between 0.5 and 10.0 g/m².

6. The steel sheet or part according to any one of claims 1 to 5, wherein the polymer is a polyester, poly-acrylic, polyurethane, polyethylene, polypropylene, or the mixtures thereof.

7. Use of the coated steel sheet or part according to any one of claims 1 to 6, for producing an enamelled steel sheet or part.

8. A process for enamelling a steel sheet or part comprising the steps consisting in:
- applying to one or both sides of a steel sheet whose composition is suitable for enamelling, a formulation layer comprising 0.008 to 5% by weight of particles of non-oxide ceramic whose melting point is above 600°C and whose average diameter D50 is between 0.01 and 3 µm, an optional solvent, the balance being a polymer which, when heated from ambient temperature to 800°C in air, gets burned at more than 80% by weight at 440°C and is completely burned at 600°C, the coating weight of said particles being between 0.001 and 0.250 g/m²,
- curing said layer so as to obtain a polymer coating in which the particles of non-oxide ceramic are homogeneously dispersed,
- optionally subjecting said coated steel sheet to a forming operation in order to obtain a part,
- applying to said polymer coating a layer of ground coat enamel, and optionally a further layer of white or light-coloured cover coat enamel, then
- subjecting said ground coat enamel and said optional white or light-coloured cover coat enamel to a firing to obtain an enamelled steel sheet or part.

9. The process according to claim 8, wherein, when the polymer is a radiation curable polymer, the formulation comprises no solvent.

10. The process according to claim 9, wherein said polymer is cured by exposure to ionizing or actinic radiation.

11. The process according to claim 8, wherein the formulation comprises a solvent, and the polymer is a thermal curable polymer.

12. The process according to claim 11, wherein said formulation comprises 0.008 to 5% by weight of said particles of non-oxide ceramic, 10 to 70% by weight of said polymer, the balance of the formulation being a solvent.

13. The process according to claim 11 or 12, wherein said steel sheet coated with said formulation layer is subjected to a heat treatment by heating it from ambient temperature to a temperature T1, and maintaining it at said temperature T1 for a time t1, so as to completely evaporate the solvent and cure the polymer.

14. The process according to claim 13, wherein said temperature T1 is between 50 and 220°C, and said time t1 is between 5 and 60 s.

## Patentansprüche

1. Stahlblech oder -teil, das auf einer oder beiden Seiten mit einer Beschichtung beschichtet ist, die aus einer Polymermatrix besteht, in der Partikel aus Nicht-Oxidkeramik homogen dispergiert sind, wobei das Beschichtungsgewicht der Partikel zwischen 0,001 und 0,250 g/m² liegt, der Schmelzpunkt der Nicht-Oxidkeramik über 600 °C liegt und der durchschnittliche Durchmesser D50 der Partikel zwischen 0,01 und 3 µm liegt, wobei die Zusammensetzung von dem Stahlblech oder -teil zum Emaillieren geeignet ist, und das Polymer, wenn es von Umgebungstemperatur auf 800 °C in der Luft erhitzt wird, bei 440 °C zu mehr als 80 Gew.-% verbrennt und bei 600 °C vollständig verbrennt.

2. Stahlblech oder -teil nach Anspruch 1, wobei das Beschichtungsgewicht von den Partikeln aus der Nicht-Oxidkeramik zwischen 0,01 und 0,10 g/m² liegt.

3. Stahlblech oder -teil nach Anspruch 1 oder 2, wobei der Schmelzpunkt der Nicht-Oxidkeramik über 700 °C liegt.

4. Stahlblech oder -teil nach einem der Ansprüche 1 bis 3, wobei die Partikel aus der Nicht-Oxidkeramik aus der Gruppe ausgewählt sind, die aus Nitriden, Boriden, Siliciden, Sulfiden, Carbiden und Mischungen daraus besteht.

5. Stahlblech oder -teil nach einem der Ansprüche 1 bis 4, wobei das Beschichtungsgewicht von der Polymerbeschichtung zwischen 0,5 und 10,0 g/m² liegt.

6. Stahlblech oder -teil nach einem der Ansprüche 1 bis 5, wobei das Polymer ein Polyester, ein Polyacrylpolymer, Polyurethan, Polyethylen, Polypropylen oder Mischungen daraus ist.

7. Verwendung des beschichteten Stahlblechs oder -teils nach einem der Ansprüche 1 bis 6 zum Herstellen von einem emaillierten Stahlblech oder -teil.

8. Verfahren zum Emaillieren von einem Stahlblech oder -teil, das die Schritte umfasst, welche aus dem Folgenden bestehen:
- Auftragen auf einer oder beiden Seiten von einem Stahlblech, dessen Zusammensetzung zum Emaillieren geeignet ist, von einer Formulierungsschicht, umfassend 0,008 bis 5 Gew.-% Partikel aus Nicht-Oxidkeramik, deren Schmelzpunkt über 600 °C liegt und deren durchschnittlicher Durchmesser D50 zwischen 0,01 und 3 µm liegt, und ein optionales Lösungsmittel, wobei der Ausgleich ein Polymer ist, das, wenn es von Umgebungstemperatur auf 800 °C in der Luft erhitzt wird, bei 440 °C zu mehr als 80 Gew.-% verbrennt und bei 600 °C vollständig verbrennt, wobei das Beschichtungsgewicht der Partikel zwischen 0,001 und 0,250 g/m² liegt,
- Härten der Schicht, um eine Polymerbeschichtung zu erhalten, in der die Partikel aus Nicht-Oxidkeramik homogen dispergiert sind,
- optionales Unterziehen von dem beschichteten Stahlblech einem Formungsarbeitsgang, um ein Teil zu erhalten,
- Auftragen auf die Polymerbeschichtung von einer Schicht aus Grundschichtemaille und optional von einer weiteren Schicht aus weißer oder leicht gefärbter Deckschichtemaille, dann
- Unterziehen von der Grundschichtemaille und der optionalen weißen oder leicht gefärbten Deckschichtemaille einem Brennvorgang, um ein emailliertes Stahlblech oder -teil zu erhalten.

9. Verfahren nach Anspruch 8, wobei, wenn das Polymer ein strahlungshärtbares Polymer ist, die Formulierung kein Lösungsmittel umfasst.

10. Verfahren nach Anspruch 9, wobei das Polymer durch Exposition zu ionisierender oder aktinischer Strahlung gehärtet wird.

11. Verfahren nach Anspruch 8, wobei die Formulierung ein Lösungsmittel umfasst und das Polymer ein thermisch härtbares Polymer ist.

12. Verfahren nach Anspruch 11, wobei die Formulierung 0,008 bis 5 Gew.-% von den Partikeln aus der Nicht-Oxidkeramik und 10 bis 70 Gew.-% von dem Polymer umfasst, wobei der Ausgleich der Formulierung ein Lösungsmittel ist.

13. Verfahren nach Anspruch 11 oder 12, wobei das Stahlblech, das mit der Formulierungsschicht beschichtet ist, einer Hitzebehandlung unterzogen wird, indem es von Umgebungstemperatur auf eine Temperatur T1 erhitzt wird und es für eine Zeit t1 auf der Temperatur T1 gehalten wird, um das Lösungsmittel vollständig zu verdampfen und das Polymer zu härten.

14. Verfahren nach Anspruch 13, wobei die Temperatur T1 zwischen 50 und 220 °C beträgt und die Zeit t1 zwischen 5 und 60 s beträgt.

## Revendications

1. Feuille ou partie d'acier revêtue sur un ou les deux côtés avec un revêtement se composant d'une matrice de polymère dans laquelle des particules de céramique sans oxyde sont dispersées de manière homogène, le poids de revêtement desdites particules étant compris entre 0,001 et 0,250 g/m², le point de fusion de ladite céramique sans oxyde étant supérieur à 600 °C, le diamètre moyen D50 desdites particules étant compris entre 0,01 et 3 µm, la composition de ladite feuille ou partie d'acier étant appropriée pour l'émaillage, et ledit polymère, lorsqu'il est chauffé de la température ambiante à 800 °C dans de l'air, brûlant à plus de 80 % en poids à 440 °C et brûlant complètement à 600 °C.

2. Feuille ou partie d'acier selon la revendication 1, dans laquelle le poids de revêtement desdites particules de céramique sans oxyde est compris entre 0,01 et 0,10 g/m².

3. Feuille ou partie d'acier selon la revendication 1 ou 2, dans laquelle le point de fusion de ladite céramique sans oxyde est supérieur à 700 °C.

4. Feuille ou partie d'acier selon l'une quelconque des revendications 1 à 3, dans laquelle lesdites particules de céramique sans oxyde sont choisies dans le groupe constitué par les nitrures, les borures, les siliciures, les sulfures, les carbures et leurs mélanges.

5. Feuille ou partie d'acier selon l'une quelconque des revendications 1 à 4, dans laquelle le poids de revêtement dudit revêtement de polymère est compris entre 0,5 et 10,0 g/m².

6. Feuille ou partie d'acier selon l'une quelconque des revendications 1 à 5, dans laquelle le polymère est un polyester, un polyacrylique, un polyuréthane, un polyéthylène, un polypropylène ou leurs mélanges.

7. Utilisation de la feuille ou de la partie d'acier revêtue selon l'une quelconque des revendications 1 à 6, pour la production d'une feuille ou d'une partie d'acier émaillée.

8. Procédé d'émaillage d'une feuille ou d'une partie d'acier comprenant les étapes consistant à :
- appliquer sur un ou les deux côtés d'une feuille d'acier dont la composition est appropriée pour l'émaillage, une couche de formulation comprenant de 0,008 à 5 % en poids de particules de céramique sans oxyde dont le point de fusion est supérieur à 600 °C et dont le diamètre moyen D50 est compris entre 0,01 et 3 µm, un solvant facultatif, le reste étant constitué d'un polymère qui, lorsqu'il est chauffé de la température ambiante à 800 °C dans de l'air, brûle à plus de 80 % en poids à 440 °C et brûle complètement à 600 °C, le poids de revêtement desdites particules étant compris entre 0,001 et 0,250 g/m²,
- durcir ladite couche de sorte à obtenir un revêtement de polymère dans lequel les particules de céramique sans oxyde sont dispersées de manière homogène,
- soumettre de manière facultative ladite feuille d'acier revêtue à une opération de formage afin d'obtenir une partie,
- appliquer sur ledit revêtement de polymère une couche d'émail de fond, et facultativement une autre couche d'un email de revêtement blanc ou légèrement coloré, puis
- cuire ledit émail de fond et ledit email de revêtement blanc ou légèrement coloré pour obtenir une feuille ou une partie d'acier émaillée.

9. Procédé selon la revendication 8, dans lequel lorsque le polymère est un polymère durcissable par rayonnement, la formulation ne comprend pas de solvant.

10. Procédé selon la revendication 9, dans lequel ledit polymère est durci par exposition à une ionisation ou à un rayonnement actinique.

11. Procédé selon la revendication 8, dans lequel la formulation comprend un solvant et le polymère est un polymère thermodurcissable.

12. Procédé selon la revendication 11, dans lequel ladite formulation comprend de 0,008 à 5 % en poids desdites particules de céramique sans oxyde, de 10 à 70 % en poids dudit polymère, le reste de la formulation étant constituée d'un solvant.

13. Procédé selon la revendication 11 ou 12, dans lequel ladite feuille en acier revêtue avec ladite couche de formulation est soumise à un traitement thermique par son chauffage de la température ambiante à une température T1, et son maintien à ladite température T1 pendant un temps t1, de sorte à totalement évaporer le solvant et durcir le polymère.

14. Procédé selon la revendication 13, dans lequel ladite température T1 est comprise entre 50 et 220 °C, et ledit temps t1 est compris entre 5 et 60 s.
